# EUROPEAN PATENT APPLICATION

(11) **EP 4 421 201 A1**
(43) Date of publication of application: **28.08.2024**
(21) Application number: 22907895.1
(22) Date of filing: 13.12.2022
(51) Int. Cl.: C22C 38/02, C22C 38/04, C22C 38/06, C22C 38/14, C22C 38/00, C22C 38/60, C21D 5/14, B21B 1/16, C21D 9/52, C21D 8/02

(54) **CALCIUM-CONTAINING GRAPHITE STEEL HAVING EXCELLENT MACHINABILITY, AND MANUFACTURING METHOD THEREFOR**

(30) Priority: 14.12.2021 KR 20210178349
(71) Applicant: POSCO Co., Ltd, Pohang-si, Gyeongsangbuk-do 37859 (KR)
(72) Inventor: CHOI, Sangwoo, Pohang-si Gyeongsangbuk-do 37664 (KR); LIM, Namsuk, Pohang-si Gyeongsangbuk-do 37669 (KR)
(74) Representative: Nederlandsch Octrooibureau
(86) International application number: PCT/KR2022/020233
(87) International publication number: WO 2023/113428

(57) **Abstract**

The present invention relates to a graphite steel having excellent machinability, and a manufacturing method therefor, and more specifically, to a calcium-containing graphite steel having machinability superior to that of normal free-cutting steel and a manufacturing method therefor.

## Description

### [Technical Field]

The present disclosure relates to a graphite steel having excellent machinability and a manufacturing method therefor, and more particularly, to a calcium-containing graphite steel having machinability superior to that of normal free-cutting steel and a manufacturing method therefor.

### [Background Art]

In general, free-cutting steels to which machinability-imparting elements such as Pb and Bi are added have been used as a material for mechanical parts that require machinability. In order to improve machinability of steel materials, liquid metal embrittlement may be used by adding low-melting point machinability-imparting elements such as Pb and Bi to steel, or a large amount of MnS may be formed in steel. Such free-cutting steels have excellent machinability of steels such as surface roughness, chip controllability, and tool life during cutting.

However, Pb-added free-cutting steel, which is generally known to have excellent machinability, is very harmful to the human body because harmful substances such as toxic fume are emitted during a cutting process and causes a problem in recycling of steel materials. Therefore, addition of S, Bi, Te, Sn, and the like is suggested for replacement thereof. However, it has been known that many problems may be caused thereby, for example, cracks easily occur while manufacturing steel materials causing considerable difficulties in production or cracks may occur during hot rolling.

Free-cutting steel developed to solve the above-described problems is graphite steel. Graphite steel, as a steel containing fine graphite grains inside a ferrite matrix or a pearlite matrix, has excellent machinability because fine graphite grains contained therein serve as a crack source during cutting, acting as a chip breaker.

However, despite these advantages of graphite steel, graphite steel has not been commercialized currently. When carbon is added to steel, graphite, even a stable phase, precipitates as cementite that is a metastable phase, so that it is difficult to precipitate graphite without a separate long-term heat treatment. During such a long-term heat treatment process, decarburization occurs, causing adverse effects on performance of final products.

In addition, although graphite grains are precipitated by graphitization heat treatment, in the case where the graphite grains are non-uniformly distributed in irregular shapes, physical properties are non-uniformly distributed during cutting to considerably deteriorate chip controllability or surface roughness and shorten tool life, making it difficult to obtain advantages of graphite steel. Therefore, there is a need to provide a method for manufacturing a graphite free-cutting steel having excellent machinability by using MnS inclusions together with graphite grains.

(Related Art Document) Patent Document 1: Korean Patent Application Publication No. 10-2015-0057400

### [Disclosure]

### [Technical Problem]

Provided are a calcium-containing graphite steel having excellent machinability and a manufacturing method therefor.

However, the technical problems to be solved by the present disclosure are not limited to the aforementioned problems, and any other technical problems not mentioned herein will be clearly understood from the following description by those skilled in the art to which the present disclosure pertains.

### [Technical Solution]

In accordance with an aspect of the present disclosure to achieve the above-described objects, a graphite steel includes, in percent by weight (wt%), 0.60 to 0.90% of carbon (C), 2.0 to 2.5% of silicon (Si), 0.7 to 1.3% of manganese (Mn), 0.2 to 0.5% of sulfur (S), 0.01 to 0.05% of aluminum (Al), 0.005 to 0.020% of titanium (Ti), 0.003 to 0.015% of nitrogen (N), 0.0001 to 0.050% of calcium (Ca), and the balance of iron (Fe) and inevitable impurities, wherein the graphite steel includes a microstructure in which graphite grains are distributed in a ferrite matrix, has a graphitization rate of 95% or more, and includes a total of 5 wt% or less of MnS inclusions and pearlite.

In accordance with another aspect of the present disclosure, a method for manufacturing a graphite steel includes: preparing a billet including, in percent by weight (wt%), 0.60 to 0.90% of carbon (C), 2.0 to 2.5% of silicon (Si), 0.7 to 1.3% of manganese (Mn), 0.2 to 0.5% of sulfur (S), 0.01 to 0.05% of aluminum (Al), 0.005 to 0.020% of titanium (Ti), 0.003 to 0.015% of nitrogen (N), 0.0001 to 0.050% of calcium (Ca), and the balance of iron (Fe) and inevitable impurities; hot rolling the billet to prepare a wire rod; and performing graphitizing heat treatment on the prepared wire rod.

### [Advantageous Effects]

Since the graphite steel according to the present disclosure includes calcium (Ca), a Ca-Al-based oxide acting as a nucleus of graphitization is formed to promote graphitization and a Ca-based emulsion is formed to improve machinability. The present disclosure may provide a graphite steel having excellent machinability and capable of replacing conventional free-cutting steels and a manufacturing method therefor.

The graphite steel according to the present disclosure having excellent machinability may replace conventional free-cutting steel materials, and thus eco-friendly graphite free-cutting steel from which harmful elements such as Pb and Bi are replaced may be provided.

### [Best Mode]

A graphite steel according to an embodiment of the present disclosure includes, in percent by weight (wt%), 0.60 to 0.90% of carbon (C), 2.0 to 2.5% of silicon (Si), 0.7 to 1.3% of manganese (Mn), 0.2 to 0.5% of sulfur (S), 0.01 to 0.05% of aluminum (Al), 0.005 to 0.020% of titanium (Ti), 0.0030 to 0.0150% of nitrogen (N), 0.0001 to 0.050% of calcium (Ca), and the balance of iron (Fe) and inevitable impurities, wherein the graphite steel includes a microstructure in which graphite grains are distributed in a ferrite matrix, has a graphitization rate of 95% or more, and includes a total of 5 wt% or less of MnS inclusions and pearlite.

### [Modes of the Invention]

Hereinafter, preferred embodiments of the present disclosure will now be described. However, the present disclosure may be embodied in many different forms and should not be construed as being limited to the embodiments set forth herein. In addition, these embodiments are provided so that this disclosure will be thorough and complete, and will fully convey the scope of the disclosure to those skilled in the art.

The terms used herein are merely used to describe particular embodiments. Thus, an expression used in the singular encompasses the expression of the plural, unless it has a clearly different meaning in the context.

Hereinafter, the unit is wt% unless otherwise stated. In addition, it is to be understood that the terms such as "including" or "having" are intended to indicate the existence of components disclosed in the specification, and are not intended to preclude the possibility that one or more other components may exist or may be added.

Meanwhile, unless otherwise defined, all terms used herein have the same meaning as commonly understood by one of ordinary skill in the art to which this disclosure belongs. Thus, these terms should not be interpreted in an idealized or overly formal sense unless expressly so defined herein. As used herein, the singular forms are intended to include the plural forms as well, unless the context clearly indicates otherwise.

In addition, the terms "about", "substantially", etc. used throughout the specification mean that when a natural manufacturing and substance allowable error are suggested, such an allowable error corresponds a value or is similar to the value, and such values are intended for the sake of clear understanding of the present invention or to prevent an unconscious infringer from illegally using the disclosure of the present invention.

Hereinafter, a graphite steel having excellent machinability and a manufacturing method therefor according to the present disclosure will be described in detail.

### [Graphite Steel]

A graphite steel according to an embodiment of the present disclosure may include, in percent by weight (wt%), 0.60 to 0.90% of carbon (C), 2.0 to 2.5% of silicon (Si), 0.7 to 1.3% of manganese (Mn), 0.2 to 0.5% of sulfur (S), 0.01 to 0.05% of aluminum (Al), 0.005 to 0.020% of titanium (Ti), 0.003 to 0.015% of nitrogen (N), 0.0001 to 0.050% of calcium (Ca), and the balance of iron (Fe) and inevitable impurities.

### [Composition]

### Carbon (C): 0.60 to 0.90 wt%

Carbon is an essential element to form graphite grains. If the C content is less than 0.60 wt%, the effect of improving machinability is insufficient and distribution of graphite is non-uniform even after graphitization is completed. On the contrary, if the C content is excessive exceeding 0.90 wt%, coarse graphite grains are formed and the aspect ratio increases, so that machinability, particularly, surface roughness, may deteriorate. Therefore, an upper limit of the C content may be controlled to 0.90 wt%.

### Silicon (Si): 2.0 to 2.5 wt%

Silicon is an essential component, as a deoxidizer, to prepare molten steel and is a graphitization-promoting element allowing carbon to precipitate into graphite by destabilizing cementite contained in steel, and thus it is preferable to necessarily include silicon. In order to achieve these effects in the present disclosure, the Si content may be 2.0 wt%.

However, if the Si content is excessive, the effects may be saturated, and hardness also increases due to sold solution strengthening effect to accelerate tool wear during cutting, embrittlement is caused by an increase in non-metallic inclusions, and excessive decarburization may occur during hot rolling. Therefore, an upper limit of the Si content may be controlled to 2.5 wt%.

### Manganese (Mn): 0.7 to 1.3 wt%

Manganese improves strength and impact properties of steel materials and combines with sulfur contained in steel to form MnS inclusions contributing to improvement of machinability. In order to achieve these effects in the present disclosure, the Mn content may be 0.7 wt% or more.

On the contrary, an excessive Mn content may inhibit graphitization to delay graphitization completion time and may increase strength and hardness to deteriorate machinability. Therefore, an upper limit of the Mn content may be 1.3 wt%.

### Sulfur (S): 0.2 to 0.5 wt%

Sulfur combines with manganese to form MnS inclusions and machinability may be improved as the MnS inclusions are formed. However, if the S content is excessive, graphitization of carbon in steel may be inhibited, S may be segregated into crystal grains to deteriorate toughness, a low-melting point emulsion may be formed to impair hot rollability, and mechanical anisotropy may be observed due to MnS stretched by rolling. Therefore, in the present disclosure, formation of MnS inclusions may be induced by adjusting the S content within a range capable of contributing to improvement of machinability without causing mechanical anisotropy.

Therefore, if the S content is controlled to less than 0.2 wt%, MnS inclusions cannot be formed in a fraction sufficient to improve machinability. In addition, if the S content exceeds 0.5 wt%, anisotropy of a material increases to cause breakage during cutting so that risks may occur during processing.

### Aluminum (Al): 0.01 to 0.05 wt%

Aluminum is the second most important material to promote graphitization after silicon. This is because aluminum, when existing as a solid solution of Al, destabilizes cementite, and thus Al needs to exist as a solid solution. In the present disclosure, Al may be contained in an amount of 0.01 wt% or more to obtain such effects.

However, if the Al content is excessive, not only the effects may be saturated but also nozzle clogging may be induced during continuous casting and AlN may be formed in austenite grain boundaries causing non-uniform distribution of graphite including AlN as nuclei in the grain boundaries. Therefore, an upper limit of the Al content may be controlled to 0.05 wt%.

### Titanium (Ti): 0.005 to 0.020 wt%

Titanium, like aluminum, combines with nitrogen to form nitrides such as TiN and AlN, and these nitrides act as nuclei for graphite formation during constant-temperature heat treatment.

While AlN that is formed at a low temperature non-uniformly precipitates after austenite is formed, TiN that is formed at a temperature higher than that of AlN is crystallized before formation of austenite is completed and thus uniformly distributed in the austenite grain boundaries and in the grains. Therefore, graphite grains formed of TiN as nuclei are also distributed finely and uniformly.

Although the Ti content may be 0.005 wt% or more to obtain these effects, addition of Ti in an amount greater than 0.02 wt% may cause consumption of carbon required for forming graphite by forming coarse carbonitrides, thereby deteriorating graphitization. Therefore, an upper limit of the Ti content may be controlled to 0.020 wt%.

### Nitrogen (N): 0.003 to 0.015 wt%

Nitrogen combines with titanium and aluminum to form TiN, AlN, and the like, and nitrides such as AlN are mainly formed in austenite grain boundaries. Because graphite is formed using such nitrides as nuclei during graphitizing heat treatment, non-uniform distribution of graphite may be caused thereby, and therefore it is necessary to add an appropriate amount thereof.

If the amount of nitrogen added is excessive, nitrogen fails to bind to a nitride-forming element and remains as a solid solution to increase strength and stabilize cementite, thereby adversely affecting to delay graphitization.

Therefore, a lower limit of the N content may be controlled to 0.003 wt% and an upper limit thereof may be controlled to 0.015 wt% in the present disclosure such that nitrogen is consumed to form nitrides acting as nuclei for forming graphite and does not remain as a solid solution.

### Calcium (Ca): 0.0001 to 0.050 wt%

Calcium forms a Ca-Al-based oxide in steel having the composition of the present disclosure, and the Ca-Al-based oxide may act as a nucleus of graphitization to promote graphitization and may also form a Ca-based emulsion to improve machinability. Stress is concentrated during a cutting process at the interface between the Ca-based emulsion and the matrix structure to form voids which grow and spread to form cracks, exhibiting the effects of being cut and separated as chips in steel.

The effects are insufficient in the case where the Ca content is less than 0.0001 wt%, and coarse oxide-based non-metal inclusions are produced in a large quantity in the case where the Ca content is greater than 0.050 wt%, thereby deteriorating fatigue strength of mechanical parts. Therefore, the Ca content may be controlled to a range of 0.0001 to 0.050 wt%.

### Other components

The remaining component of the composition of the present disclosure is iron (Fe). However, the composition may include unintended impurities inevitably incorporated from raw materials or surrounding environments in normal manufacturing processes. However, the graphite steel according to the present disclosure may not include phosphorus (P) or oxygen (O). These impurities are not specifically mentioned in the present disclosure, as they are known to any person skilled in the art.

### [Microstructure]

The graphite steel according to the present disclosure has a microstructure in which graphite grains are distributed in a ferrite matrix, has a graphitization rate of 95% or more, and includes a total of 5 wt% or less of MnS inclusions and pearlite.

The graphite steel according to an embodiment of the present disclosure may have a graphitization rate of 98% or more, more preferably 99% or more, and most preferably 99.5% or more.

Meanwhile, the graphitization rate refers to a ratio of an amount of carbon existing as a graphite state to an amount of carbon added to steel and is defined by Equation 1 below. A graphitization rate of 95% or more indicates that most carbon added to the steel is consumed to form graphite (in which amounts of carbon as solid solutions contained in ferrite and in fine carbides are extremely small and thus not considered) and the graphite steel has a microstructure in which graphite grains are distributed in a ferrite matrix in which undegraded pearlite does not exist. Graphitization rate (%) = (1-amount of C in undergraded pearlite/amount of C in steel) × 100
(Here, the graphitization rate is 100% in the case where there is no undegraded pearlite)

All of the descriptions given above with reference to the graphite steel may be applied to a method for manufacturing a graphite steel to be described below. Although duplicate descriptions may be omitted, the omitted descriptions may also be applied thereto in the same manner.

### [Method for Manufacturing Graphite Steel]

A method for manufacturing a graphite steel according to another embodiment of the present disclosure includes: preparing a billet including, in percent by weight (wt%), 0.60 to 0.90% of carbon (C), 2.0 to 2.5% of silicon (Si), 0.7 to 1.3% of manganese (Mn), 0.2 to 0.5% of sulfur (S), 0.01 to 0.05% of aluminum (Al), 0.005 to 0.02% of titanium (Ti), 0.0030 to 0.0150% of nitrogen (N), 0.0001 to 0.05% of calcium (Ca), and the balance of iron (Fe) and inevitable impurities; hot rolling the billet to prepare a wire rod; and performing graphitizing heat treatment on the prepared wire rod.

### Rolling Process

In addition, according to an embodiment of the present disclosure, the hot rolling may include hot rolling in a temperature range of 900 to 1150°C. Specifically, the hot rolling may be performed by hot rolling after conducting heat treatment in a temperature range of 900 to 1150°C for a certain period of time.

The rolling temperature of the wire rod may be controlled in the range of 900 to 1150°C because surface defects easily occur or a rolling load increases during hot rolling at a temperature lower than 900°C making a rolling process difficult, and austenite grain size (AGS) increases at a temperature higher than 1150°C so that graphitizing heat treatment time increases after hot rolling the wire rod.

### Graphitizing Heat Treatment Process

In addition, according to an embodiment of the present disclosure, the graphitizing heat treatment may include heat treatment in a temperature range of 700 to 800°C for 5 hours or more, preferably, for 5 hours to 20 hours.

If the wire rod is heat-treated in a temperature range of 700 to 800°C for 5 hours or more, the graphitization rate may be 95% or more. However, at a temperature lower than 700°C, graphitizing heat treatment time increases to exceed 20 hours. At a temperature higher than 800°C, not only graphitizing heat treatment time increases, but also austenite is formed by reverse-transformation of pearlite and pearlite may be formed during cooling. Thus, they are not desirable.

Hereinafter, the present disclosure will be described in more detail with reference to the following examples.

These embodiments are provided to fully convey the scope of the disclosure to those skilled in the art. The present disclosure may, however, be embodied in many different forms and should not be construed as limited to the exemplary embodiments set forth herein.

### [Examples]

Billets having compositions shown Table 1 below were maintained at a heating temperature of 1050°C for 90 minutes and rolled at a high speed to prepare wire rods having a diameter of 19 mm. In this regard, graphitizing heat treatment times and graphitization rates are shown in Table 2. In addition, graphitizing heat treatment was performed by constantly applying "Al temperature - 50°C" as a graphitizing heat treatment temperature.

In Tables 1 and 2 below, Examples 1 to 11 show graphite steel wire rods satisfying the composition range of alloying elements and manufacturing conditions of the present disclosure, and Comparative Examples 1 to 7 show wire rods not satisfying the composition range of alloying elements and/or manufacturing conditions of the present disclosure.

**[Table 1]**

| Category | Composition of alloying elements (wt%) | | | | | | | |
|---|---|---|---|---|---|---|---|---|
| | C | Si | Mn | S | Al | Ti | N | Ca |
| Example 1 | 0.67 | 2.1 | 0.85 | 0.31 | 0.015 | 0.015 | 0.005 | 0.010 |
| Example 2 | 0.85 | 2.15 | 0.96 | 0.24 | 0.023 | 0.017 | 0.008 | 0.020 |
| Example 3 | 0.72 | 2.35 | 1.07 | 0.35 | 0.043 | 0.007 | 0.010 | 0.015 |
| Example 4 | 0.68 | 2.18 | 1.16 | 0.45 | 0.035 | 0.009 | 0.009 | 0.030 |
| Example 5 | 0.82 | 2.25 | 0.95 | 0.35 | 0.040 | 0.012 | 0.014 | 0.040 |
| Example 6 | 0.62 | 2.48 | 0.80 | 0.25 | 0.042 | 0.006 | 0.012 | 0.045 |
| Example 7 | 0.73 | 2.42 | 1.20 | 0.30 | 0.034 | 0.011 | 0.006 | 0.035 |
| Example 8 | 0.78 | 2.32 | 1.25 | 0.43 | 0.019 | 0.016 | 0.008 | 0.030 |
| Example 9 | 0.85 | 2.15 | 0.95 | 0.27 | 0.027 | 0.009 | 0.013 | 0.025 |
| Example 10 | 0.75 | 2.26 | 1.15 | 0.26 | 0.030 | 0.018 | 0.007 | 0.015 |
| Example 11 | 0.73 | 2.46 | 1.20 | 0.42 | 0.020 | 0.008 | 0.008 | 0.035 |
| Comparative | 0.63 | 2.00 | 1.35 | 0.05 | 0.005 | 0.016 | 0.001 | 0.060 |

| Example 1 | | | | | | | | |
|---|---|---|---|---|---|---|---|---|
| Comparative Example 2 | 0.68 | 2.20 | 1.41 | 0.13 | 0.006 | 0.020 | 0.002 | 0.065 |
| Comparative Example 3 | 0.73 | 2.25 | 1.50 | 0.56 | 0.075 | 0.009 | 0.018 | 0.080 |
| Comparative Example 4 | 0.95 | 2.15 | 0.40 | 0.11 | 0.060 | 0.018 | 0.020 | 0.070 |
| Comparative Example 5 | 0.55 | 2.60 | 0.56 | 0.60 | 0.003 | 0.025 | 0.025 | 0.100 |
| Comparative Example 6 | 0.80 | 2.75 | 0.65 | 0.15 | 0.065 | 0.030 | 0.021 | 0.085 |
| Comparative Example 7 | 0.75 | 2.80 | 0.60 | 0.10 | 0.060 | 0.002 | 0.022 | 0.070 |

**[Table 2]**

| Category | Graphitizing Heat Treatment | | Machinability (%) |
|---|---|---|---|
| | Hour (hr) | Graphitization rate (%) | |
| Example 1 | 6.0 | 99 | 100 |
| Example 2 | 9.5 | 99 | 100 |
| Example 3 | 11.0 | 100 | 100 |
| Example 4 | 6.5 | 100 | 100 |
| Example 5 | 13.5 | 100 | 100 |
| Example 6 | 5.5 | 99.5 | 100 |
| Example 7 | 16.5 | 100 | 100 |
| Example 8 | 8.2 | 98.5 | 100 |
| Example 9 | 18.5 | 100 | 100 |
| Example 10 | 5.7 | 98 | 100 |
| Example 11 | 12.5 | 99 | 100 |
| Comparative Example 1 | 3.5 | 86 | 88 |
| Comparative Example 2 | 2.0 | 85 | 80 |
| Comparative Example 3 | 3.0 | 86 | 89 |
| Comparative Example 4 | 4.5 | 84 | 92 |
| Comparative Example 5 | 2.5 | 91 | 84 |
| Comparative Example 6 | 3.0 | 92 | 93 |
| Comparative Example 7 | 4.5 | 90 | 90 |

In Table 2, a (100%-graphitization rate) structure consists of MnS inclusions, pearlite, and some common inclusions, and a graphitized structure consists of ferrite and graphite grains.

In Table 2, machinability is a value based on machinability of common free-cutting steels (100% refers to an equivalent level).

It may be confirmed that graphitization fraction and machinability may be achieved under the conditions for manufacturing graphite free-cutting steel as shown in Table 2.

Hereinafter, Examples and Comparative Examples will be evaluated with reference to Tables 1 and 2.

In Examples 1 to 11, it was confirmed that the graphitization rates were not less than 98.5% and machinability was 100% of that of lead free-cutting steels because the compositions of alloying elements and manufacturing conditions of the present disclosure were satisfied.

On the contrary, according to Comparative Examples 1 to 7 in which Ca contents exceed 0.05 wt% in the compositions of alloying elements and graphitizing heat treatment was maintained for less than 5 hours, it was confirmed that the graphitization rates were not more than 92% and machinability was also not more than 95%.

Specifically, in the graphite steels according to Comparative Examples 1 and 2 including greater than 1.3 wt% of Mn, less than 0.2 wt% of S, and greater than 0.05 wt% of Ca, machinability was only 88% and 95% of that of lead free-cutting steels due to insufficient formation of MnS inclusions and the graphitization rates were not more than 86% because graphitizing heat treatment was maintained for 3.5 hours or less.

In addition, in the graphite steel of Comparative Example 3 including 1.50 wt% of Mn, 0.56 wt% of S, and 0.08 wt% of Ca, machinability was only 89% of that of lead free-cutting steel and the graphitization rate was only 86% because graphitizing heat treatment was maintained for 3.0 hours.

In addition, in the graphite steel of Comparative Example 4 including 0.95 wt% of C, 0.40 wt% of Mn, 0.011 wt% of S, and 0.07 wt% of Ca, machinability was only 92% of that of lead free-cutting steels and the graphitization rate was only 84% because graphitizing heat treatment was maintained for 4.5 hours.

In addition, in the graphite steel of Comparative Example 5 including 0.55 wt% of C, 2.6 wt% of Si, 0.56 wt% of Mn, 0.60 wt% of S, 0.025 wt% of TI, and 0.1 wt% of Ca, machinability was only 91% of that of lead free-cutting steels and the graphitization rate was only 91% because graphitizing heat treatment was maintained for 2.5 hours.

In addition, in the graphite steel of Comparative Example 6 including 2.7 wt% of Si, 0.65 wt% of Mn, 0.15 wt% of S, 0.03 wt% of Ti, and 0.085 wt% of Ca, machinability was only 93% of that of lead free-cutting steels and the graphitization rate was only 92% because graphitizing heat treatment was maintained for 3.0 hours.

In addition, in the graphite steel of Comparative Example 7 including 2.8 wt% of Si, 0.60 wt% of Mn, 0.10 wt% of S, 0.002 wt% of Ti, and 0.07 wt% of Ca, machinability was only 90% of that of lead free-cutting steels and the graphitization rate was only 90% because graphitizing heat treatment was maintained for 4.5 hours.

While the present disclosure has been particularly described with reference to exemplary embodiments, it should be understood by those of skilled in the art that various changes in form and details may be made without departing from the spirit and scope of the present disclosure.

### [Industrial Applicability]

According to the present disclosure, the graphite free-cutting steel according to the present disclosure having excellent machinability may replace conventional free-cutting steels and may be eco-friendly by replacing harmful substances such as Pb and Bi, and therefore the present disclosure has industrial applicability.

## Claims

1. A graphite steel comprising, in percent by weight (wt%), 0.60 to 0.90% of carbon (C), 2.0 to 2.5% of silicon (Si), 0.7 to 1.3% of manganese (Mn), 0.2 to 0.5% of sulfur (S), 0.01 to 0.05% of aluminum (Al), 0.005 to 0.020% of titanium (Ti), 0.003 to 0.015% of nitrogen (N), 0.0001 to 0.050% of calcium (Ca), and the balance of iron (Fe) and inevitable impurities,
wherein the graphite steel includes a microstructure in which graphite grains are distributed in a ferrite matrix, has a graphitization rate of 95% or more, and includes a total of 5 wt% of MnS inclusions and pearlite.

2. The graphite steel according to claim 1, wherein the graphite steel has a graphitization rate of 99% or more.

3. The graphite steel according to claim 1, wherein the graphite steel does not include at least one phosphorus (P) and oxygen (O).

4. A method for manufacturing a graphite steel, the method comprising:
preparing a billet including, in percent by weight (wt%), 0.60 to 0.90% of carbon (C), 2.0 to 2.5% of silicon (Si), 0.7 to 1.3% of manganese (Mn), 0.2 to 0.5% of sulfur (S), 0.01 to 0.05% of aluminum (Al), 0.005 to 0.020% of titanium (Ti), 0.003 to 0.015% of nitrogen (N), 0.0001 to 0.05% of calcium (Ca), and the balance of iron (Fe) and inevitable impurities;
hot rolling the billet to prepare a wire rod; and
performing graphitizing heat treatment on the prepared wire rod.

5. The method according to claim 4, wherein the hot rolling comprises hot rolling in a temperature range of 900°C to 1150°C.

6. The method according to claim 4, wherein the graphitizing heat treatment comprises heat treatment in a temperature range of 700°C to 800°C for 5 hours or more.

7. The method according to claim 6, wherein the graphitizing heat treatment is performed for 5 hours to 20 hours.
